

## [54] PROCESSING COPPER BASE ALLOYS

[76] Inventors: **Richard Dale Smith**, 51 Twin Cones Rd., Madison, Conn. 06443; **Irwin Broverman**, 7337/B S. Shore Dr., Apt. 1017, Chicago, Ill. 60649

[22] Filed: July 24, 1972

[21] Appl. No.: 274,807

## Related U.S. Application Data

[60] Division of Ser. No. 115,839, Feb. 16, 1971, abandoned, which is a continuation of Ser. No. 800,354, Feb. 10, 1969, abandoned, which is a continuation of Ser. No. 530,942, March 1, 1966, abandoned.

[52] U.S. Cl..... 148/11.5 R

[51] Int. Cl..... C22f 1/08

[58] Field of Search..... 148/11.5 R, 12.7

## [56] References Cited

## UNITED STATES PATENTS

2,011,259 8/1935 Price ..... 75/157.5

|           |         |                  |            |
|-----------|---------|------------------|------------|
| 2,101,087 | 12/1937 | Munson .....     | 75/157.5   |
| 2,365,208 | 12/1944 | Morris.....      | 148/11.5 R |
| 3,146,095 | 8/1964  | Hechinger.....   | 75/157.5   |
| 3,663,311 | 5/1972  | Chin et al. .... | 148/11.5 R |

## FOREIGN PATENTS OR APPLICATIONS

578,873 7/1946 Great Britain ..... 75/157.5

Primary Examiner—W. W. Stallard

Attorney, Agent, or Firm—Robert H. Bachman

[57]

## ABSTRACT

A process for obtaining improved strength properties and improved stress corrosion resistance in copper base alloys including the steps of hot rolling, annealing, cold rolling, and stress relief annealing.

3 Claims, 2 Drawing Figures



PATENTED JUN 11 1974

3,816,187



## PROCESSING COPPER BASE ALLOYS

## CROSS REFERENCE TO RELATED APPLICATIONS

This application is a division of application Ser. No. 115,839, filed Feb. 16, 1971, by Richard Dale Smith and Irwin Broverman for "Copper Base Alloys," now abandoned, which in turn is a Continuation of application Ser. No. 800,354, filed Feb. 10, 1969, by Richard Dale Smith and Irwin Broverman for "Copper Base Alloys," now abandoned, which in turn is a Continuation of application Ser. No. 530,942, filed Mar. 1, 1966, by Richard Dale Smith and Irwin Broverman for "Copper Base Alloys," now abandoned.

The present application relates to new and improved copper base alloys. More particularly, the present invention resides in greatly improved copper base alloys containing zinc, aluminum and nickel, said alloys having greatly improved physical properties and being suitable for a wide range of applications, including castings, forgings, extrusions, and hot or cold rolled or drawn products. The improved alloys of the present invention are particularly suitable for use in wrought products.

Over the years, numerous attempts have been made to improve the strength characteristics of ductile brass without sacrifice of formability. These attempts have concentrated on utilizing a great variety of alloying additions in order to achieve this goal. Some of these alloying additions are quite expensive and add considerably to the cost of the alloy.

In addition, the art has thoroughly explored many unusual thermo-mechanical processes in order to improve the strength characteristics without sacrificing formability.

The high strength brasses which have been developed in the art generally are multiphase alloys having limited ductility and cold formability. Such alloys are most suitable for application as castings or hot worked products.

Despite these extensive investigations, 70/30 brass has prevailed over the years as the best and most economical copper base alloy for severe forming applications.

Accordingly, it is a principal object of the present invention to provide an improved copper base alloy.

It is an additional object of the present invention to provide a copper base alloy having improved strength levels in either the fully annealed or cold worked tempers.

It is an additional object of the present invention to provide improved copper base alloys as aforesaid which achieve improved strength characteristics with minimal sacrifice in formability.

It is an additional object of the present invention to provide an improved copper base alloy as aforesaid, said alloy being characterized by relatively low cost so that it is economically suitable on a large scale.

Further objects and advantages of the present invention will appear hereinafter.

In accordance with the present invention, it has now been found that the foregoing objects may be readily and conveniently achieved. The improved alloy of the present invention consists essentially of the following ingredients in the following ranges, wherein all percentages are weight percentages: copper from 66 to 80.0

percent, zinc from 15.0 to 32.5 percent, aluminum from 1.5 to 5.0 percent, and nickel from 0.2 to 5 percent.

It has been found that the foregoing alloy achieves 5 greatly improved physical properties with minimal sacrifice in formability. For example, the improved alloy of the present invention has yield strength characteristics in the fully annealed condition on the order of 45,000 psi and over; whereas conventional copper base 10 alloys for forming applications normally achieve yield strengths in the fully annealed condition in the range of 10,000 to 25,000 psi and rarely over 30,000 psi. The alloys of the present invention have correspondingly 15 high yield strengths in the cold worked temper, for example, 90,000 psi and over after 50 percent cold reduction; whereas conventional alloys normally fall in the range of 50,000 to 75,000 psi.

In addition, and importantly the alloys of the present 20 invention are characterized by a high formability. Using the highly formable 70/30 brass as a standard, the alloys of the present invention have comparable formability. This is particularly surprising in view of the high strength of the alloys of the present invention.

These surprising characteristics in an inexpensive 25 alloy are particularly unexpected in view of the extensive art in this field attempting to approximate these characteristics.

The alloys of the present invention are known as 30 modified aluminum-brasses and basically have either of the following structures: (1) an alpha (face-centered cubic) structure; or (2) an alpha plus a limited amount of beta (body-centered cubic) structure.

The addition of aluminum to copper-zinc alloys has 35 long been known for its strengthening effect on such alloys. The disadvantage of the aluminum addition is that in saturated alpha phase alloys, which have highest strengths, small variation in aluminum content generally results in large variations in ductility and strength. 40 These large variations are a result of the structure of the saturated alloy changing markedly with aluminum content. For example a change in aluminum content of one percent may cause an increase in beta phase content of up to 33 percent.

In accordance with the present invention it has been 45 surprisingly found that the addition of nickel in the range of 0.2 to 5 percent by weight overcomes the disadvantages of the ternary copper-aluminum-zinc alloys such that properties and structure are more uniform over a practical range of aluminum content. In addition, a very marked grain refining effect occurs upon the addition of nickel, which is highly advantageous.

In accordance with the present invention the alloying 50 ingredients must critically fall within the foregoing ranges. The copper content must fall within the range of 66 to 80 percent by weight and preferably from 70 to 76 percent by weight. Below 66 percent by weight the strength falls off markedly and above 76 percent by weight in saturated alloys an additional phase, termed gamma having a complex cubic crystal structure, may be encountered which limits the ductility of the alloy.

Similarly, the zinc content is within the range of 15.0 55 to 32.5 percent by weight and preferably from 21 to 28 percent. The aluminum content should be maintained in the range from 1.5 to 5.0 percent by weight and preferably 2.5 to 4.5 percent and the nickel content should

be maintained in the range 0.2 to 5 percent and preferably 0.4 to 2.0 percent.

For maximum ductility-formability at any given copper-aluminum level, the nickel content should be between 0.2 and 1.0 percent while for greater strength and lesser ductility the nickel may approach higher levels up to 5 percent. At higher nickel levels ductility is reduced to such an extent that usefulness as a wrought product is impaired.

In general, the lower nickel content alloys are high strength, high ductility materials; whereas the higher nickel content alloys provide even higher strengths, but lower ductility.

The composition of specific alloys within the above ranges are subject to the further internal restriction that at about the 71.5 percent level of copper the aluminum content should preferably be in the range of 1.5 to 4.0 percent in order to insure high ductility-strength characteristics and at about the 74 percent level of copper the aluminum content should preferably be between 2.5 and 5.0 percent for the same reasons. Proportionate adjustments of aluminum content for the various copper contents between the specified limits should preferably be made.

Furthermore, in order to attain the preferred properties the aluminum content should preferably be related to the zinc content in accordance with the following equation:

$$\text{Weight \% Al} = -0.30 \text{ wt\% Zn} + 10.3 \pm 1.25$$

The subject alloys are represented in the attached drawings which are isothermal (932°F), constant nickel (0.5%) sections of the quaternary phase diagram. FIG. 1 shows the relative location of the alloys of the present invention on the ternary phase diagram. FIG. 2 shows the shaded section of FIG. 1. In FIGS. 1 and 2 the solid line represents the alpha phase boundary. In FIG. 2, the dotted line represents the alloys of the present invention at constant 0.5 percent nickel. Similar diagrams may be readily constructed for other nickel levels.

The structure of the alloys of the present invention in the cold worked and annealed condition is either (1) a matrix of fine grained, face-centered cubic, alpha phase (saturated or very nearly so), or (2) saturated alpha plus beta phase, with both structure (1) and structure (2) having very fine intermetallic compound and/or precipitate particles dispersed throughout.

The alloys of the present invention may include in addition to the foregoing materials conventional impurities typically found in commercial copper base alloys. In addition, various other alloying ingredients may be added to achieve particularly desirable results. Common impurities may include: lead; tin; phosphorus; iron; manganese; and silicon. For minimizing dezincification in corrosive environments, the addition of arsenic, antimony or phosphorus may be desirable in an amount from 0.02 to 0.10 percent.

In general, the alloys of the present invention have an alpha plus particulate phase or an alpha plus beta plus particulate phase structure and are utilizable in a wide variety of applications. In view of their high strength and high formability, they are preferably provided in the wrought form. The oxidation resistance and castability of the alloys of the present invention are excellent suggesting wide spread application as high strength, low cost foundry alloys while their excellent hot forming properties also make them desirable for forgings as

well as extrusions. In general, better combinations of mechanical properties at low costs are obtainable with the alloys of the present invention than are available in any currently produced copper base alloys regardless of price.

Processing of the subject alloys requires no unusual treatment. As an example, the processing to sheet is as follows. Melting and casting are performed under similar conditions as brass alloys. Direct chill (DC) casting is particularly suitable. Hot rolling is easily accomplished using normal brass mill procedures. Under rapid cooling conditions a non-equilibrium structure may be obtained which reduces initial cold rollability. This may be overcome by an anneal in the range of 1000° to 1200°F wherein practically equilibrium proportions of alpha and beta phases are attained.

It has been observed in the processing of the subject alloys that they exhibit an unusually high response to low temperature stress relief annealing following cold working. Normally, copper base alloys which have been heavily cold worked may respond with an increase in yield strength of up to 15 percent when annealed at temperatures below the recrystallization temperature. This increase also normally is of practical consequence only within a relatively narrow range of annealing temperatures (50° to 100°F). In the alloys of this invention, increases in yield strength of 30 to 40 percent have been noted upon low temperature annealing of material cold rolled 50 percent. Further, this response occurs over a wider range of temperature (150° to 200°F span), thereby increasing its commercial applicability. The magnitude of improvement in strength properties will be illustrated in the examples which form a part of the present specification.

A further outstanding characteristic of the subject alloys is a very marked improvement in stress corrosion resistance. The copper-zinc brasses are highly susceptible to stress corrosion cracking when exposed to certain corrosive environments. This susceptibility is proportional to zinc content and hence alloys containing more than 15% zinc are rarely chosen for stressed applications in corrosive environments. It has been found that the nickel modified aluminum brasses have greatly improved resistance to stress corrosion cracking when compared with the binary copper-zinc alloys. This behavior will be apparent from the ensuing examples. Coupled with this stress corrosion resistance is a high level of resistance to general corrosion.

The present invention will be more readily understandable from a consideration of the following illustrative examples.

#### EXAMPLE I

Alloys having the compositions listed below were prepared from cathode copper, slab zinc, nickel metal, and aluminum metal pellets. Preparation followed the ensuing sequence. Cathode copper chunks and nickel chunks were melted under charcoal, the desired aluminum content was added and stirred in, zinc chunks were added and stirred in. The melt at a temperature of about 2000°F was poured into a cast iron mold and allowed to solidify.

The resulting ingots were reheated to 1500° to 1650°F and hot rolled from 1.750 to 0.300 inch, finishing at about 1000°F. Material was then cold rolled to 0.120 inch, annealed at 1000°F for one hour, cold rolled to 0.060 inch, annealed at 1000°F for one hour

and cold rolled to 0.030 inch. Material was evaluated in the final 50 percent cold rolled condition at 0.030 inch and also in the annealed condition where various temperatures were used.

For comparative purposes, commercial 70/30 brass and a copper-aluminum-zinc alloy were subjected to the same treatment, except that the 70/30 brass was interannealed at 800°F instead of 1000°F.

The properties are given in the following table, i.e., yield strength at 0.1 percent offset, tensile strength and percent elongation both in the cold rolled and annealed tempers.

Table I

| Alloy | Composition<br>wt %       | Cold Rolled 50%          |                          |                       | Annealed 1000°F, 1 hour  |                          |                       |
|-------|---------------------------|--------------------------|--------------------------|-----------------------|--------------------------|--------------------------|-----------------------|
|       |                           | Yield<br>Strength<br>psi | Yield<br>Strength<br>psi | Percent<br>Elongation | Yield<br>Strength<br>psi | Yield<br>Strength<br>psi | Percent<br>Elongation |
| I     | 75.9Cu 19.4Zn 4.0Al 0.7Ni | 95,500                   | 124,000                  | 1.7                   | 49,500                   | 79,000                   | 38                    |
| II    | 74.2Cu 21.8Zn 3.5Al 0.5Ni | 86,000                   | 125,000                  | 2.0                   | 49,000                   | 78,000                   | 36.5                  |
| III   | 71.3Cu 21.7Zn 4.0Al 3.0Ni | 91,000                   | 128,000                  | 2.0                   | 62,000                   | 89,000                   | 26                    |
| IV    | 72.0Cu 25.0Zn 2.5Al 0.5Ni | 91,000                   | 122,000                  | 3.0                   | 53,000                   | 83,000                   | 34                    |
| V     | 76Cu 20Zn 4Al             | 89,000                   | 114,000                  | 2.0                   | 27,000                   | 65,000                   | 57                    |
| VI    | 70Cu 30Zn                 | 74,500                   | 90,000                   | 3.5                   | *41,000                  | 72,000                   | 39                    |
|       |                           |                          |                          |                       | *21,800                  | 53,000                   | 50                    |

\* — Annealed at 800°F

## EXAMPLE II

Alloy V from Example I was given the following treatment after the final cold roll: 1 hour anneal at 375°F. The properties were as follows:

5

10

Resistance to stress corrosion cracking is of importance in many applications. The improved alloys of the present invention have demonstrated a marked superiority over common brasses in this respect. In an accel-

## EXAMPLE IV

erated test in a solution containing  $(\text{NH}_4)_2(\text{SO}_4)$ ,  $\text{Cu}(\text{SO}_4)$ , and  $\text{NH}_4\text{OH}$ , highly stressed strip samples resisted cracking far beyond the abilities of 70/30 brass or 85/15 brass. These results are summarized in Table IV along with some incomplete data on resistance to stress corrosion cracking in industrial atmospheres.

Table IV

| Alloy               | Time to Failure in<br>Accelerated Test or<br>Amount of relaxation<br>in 500 Hrs. | Time to Failure<br>in Atmosphere |
|---------------------|----------------------------------------------------------------------------------|----------------------------------|
| I                   | 14% relaxation 500 hrs.                                                          | No failures at 4 mos.            |
| II                  | 43% relaxation 500 hrs.                                                          | no failures at 10 mos.           |
| VI<br>(70/30 brass) | complete failure 4 hrs.                                                          | 8 to 15 weeks                    |
| 85/15 brass         | complete failure 48-72 hrs.                                                      | no failures at 12 mos.           |

Table II

| Cold Rolled 50%                 | Cold Rolled 50% +<br>1 hour at 375°F |
|---------------------------------|--------------------------------------|
| Yield Strength<br>91,000 psi    | 114,500 psi                          |
| Tensile Strength<br>128,000 psi | 132,000 psi                          |
| Elongation<br>2.0%              | 1.2%                                 |

## EXAMPLE III

Several of the alloys prepared in Example I were evaluated for formability using two common measurements, i.e., limiting draw ratio determination for evaluating deep drawability, and Olsen cup testing to check stretch formability. These results show the improved alloys of the present invention to be nearly equivalent in drawability to 70/30 brass (listed for comparison) and only slightly less formable in stretch forming than 70/30 brass.

50 This invention may be embodied in other forms or carried out in other ways without departing from the spirit or essential characteristics thereof. The present embodiment is therefore to be considered as in all respects illustrative and not restrictive, the scope of the invention being indicated by the appended claims, and all changes which come within the meaning and range of equivalency are intended to be embraced therein.

55 55 What is claimed is:

1. A process for obtaining improved strength properties and improved stress corrosion resistance in copper base alloys consisting essentially of copper from 66 to 76 percent by weight, zinc from 15.0 to 32.5 percent by weight, aluminum from 2.5 to 4.5 percent by weight and nickel from 0.2 to 5.0 percent by weight, consisting essentially of the steps of:

- A. hot rolling said alloy at a temperature of from 1000° to 1650°F;
- B. annealing said alloy at a temperature of from 1000° to 1200°F;

- C. cold rolling at least 50 percent; and
  - D. stress relief annealing the cold worked material at a temperature below the recrystallization temperature.
2. A process according to claim 1 wherein said copper base alloy contains a material selected from the

group consisting of arsenic, phosphorus and antimony in an amount from 0.02 to 0.10 percent by weight.

- 3. A process according to claim 1 wherein said material is stress relief annealed at a temperature of 375°F for one hour.

\* \* \* \* \*

10

15

20

25

30

35

40

45

50

55

60

65

UNITED STATES PATENT OFFICE  
CERTIFICATE OF CORRECTION

Patent No. 3,816,187 Dated June 11, 1974

Inventor(s) Richard Dale Smith and Irwin Broverman

It is certified that error appears in the above-identified patent  
and that said Letters Patent are hereby corrected as shown below:

In the heading, after "Richard Dale Smith, 51 Twin  
Cones Rd., Madison, Conn. 06443; Irwin Broverman, 7337/B  
S. Shore Dr., Apt. 1017, Chicago, Ill. 60649" insert  
---assignors to Olin Mathieson Chemical Corporation, a  
corporation of Virginia---.

Signed and sealed this 29th day of October 1974.

(SEAL)

Attest:

McCoy M. GIBSON JR.  
Attesting Officer

C. MARSHALL DANN  
Commissioner of Patents